# EUROPEAN PATENT SPECIFICATION

(11) **EP 3 601 714 B1**
(45) Date of publication and mention of the grant of the patent: **28.08.2024**
(21) Application number: 18716452.0
(22) Date of filing: 20.03.2018
(51) Int. Cl.: E21B 17/042, C22C 9/06, F16L 15/00

(54) **COUPLINGS FOR WELL PUMPING COMPONENTS**
KUPPLUNGEN FÜR BOHRLOCHPUMPKOMPONENTEN
ACCOUPLEMENTS POUR ÉLÉMENTS DE POMPAGE DE PUITS

(30) Priority: 20.03.2017 US 201762473792 P
(43) Date of publication of application: 05.02.2020
(73) Proprietor: Materion Corporation, Mayfield Heights, OH 44124 (US)
(72) Inventor: NIELSEN JR., William D., Mayfield Heights, Ohio 44124 (US); NIELSEN, Diane M., Mayfield Heights, Ohio 44124 (US)
(74) Representative: Kador & Partner Part mbB
(86) International application number: PCT/US2018/023385
(87) International publication number: WO 2018/175456

(56) References cited:
- WO-A1-2015/187217
- US-A- 4 822 201
- US-A1- 2006 273 601
- US-A1- 2014 311 633
- US-A1- 2015 267 477
- NONE NONE: "Precision International Material Cat.", 31 July 2014 (2014-07-31), pages 1 - 74, XP055805604, Retrieved from the Internet <URL:http://www.totaldepthwarehouse.com/docs/precision/Precision%20Catalog.pdf> [retrieved on 20140731]
- S. ILANGOVAN ET AL: "EFFECTS OF TIN ON HARDNESS, WEAR RATE AND COEFFICIENT OF FRICTION OF CAST CU-NI-SN ALLOYS", JOURNAL OF ENGINEERING SCIENCE AND TECHNOLOGY, 1 February 2013 (2013-02-01), pages 34 - 43, XP055480063, Retrieved from the Internet <URL:http://jestec.taylors.edu.my/Vol%208%20Issue%201%20February%2013/Vol_8_1_034-043_S.%20ILANGOVAN.pdf>
- W.RAYMOND CRIBB ET AL: "Performance Advances in Copper-Nickel-Tin Spinodal Alloys", ADVANCED MATERIALS & PROCESSES, 1 September 2013 (2013-09-01), pages 20 - 25, XP055328169, Retrieved from the Internet <URL:http://www.asminternational.org/documents/10192/6019612/amp17109p20.pdf/98b04493-eab6-41dc-bee1-abcd4e64bdb3> [retrieved on 20161212]

## Description

### BACKGROUND

The present disclosure relates to couplings made from a spinodally-hardened copper alloy. The couplings are particularly useful for connecting components of a sucker rod string to a downhole pump. The alloys preferably have a sliding coefficient of friction of less than 0.4 when measured against carbon steel.

Hydrocarbon extraction apparatuses typically include a downhole pump for extracting hydrocarbons from an underground reservoir, a power source for providing power to the pump, and a sucker rod lift system connecting the power source and the downhole pump. The sucker rod lift system includes a series of sucker rods that are joined together by couplings. The rods and couplings are joined by a pin-and-box threaded connection. Additional couplings with threaded connections are also used when joining the sucker rod lift system to the downhole pump. Damage to threaded connections due to galling (wear due to adhesion between sliding surfaces) can compromise the mechanical integrity of the joint and lead to failure of the connection between the power source and the pump. In addition, the hydrocarbon extraction system operates within a conduit. Damage to the conduit and the coupling caused by repetitive contact between the outer surface of the couplings / pump and the inner surface of the conduit can compromise the mechanical integrity of the conduit or the coupling, leading either to leakage of the hydrocarbons carried by the conduit into the environment or separation of the coupling connection to the sucker rod string. Either event effectively stops the pumping process and often leads to very costly additional operations to remediate such failures.

Desired characteristics of couplings used in such systems include high tensile strength, high fatigue strength, high fracture toughness, galling resistance, and corrosion resistance. Conventional couplings are typically comprised of steel or nickel alloys which lack the full complement of preferred intrinsic characteristics, particularly galling resistance. Expensive surface treatments are typically used to increase wear resistance on couplings made from steel or nickel alloys, as well as on the inside of the conduit inside which the coupling is disposed. These surface treatments eventually wear off, and must be re-applied periodically over the course of the lifetime of the parts in order to be effective. Furthermore, while coatings may reduce wear of the component on which they are applied, the coatings are often incompatible with the other components of the system with which the coating may come into contact.

Patent application having publication number WO2015187217 discloses cold worked and spinodally-hardened copper alloy comprising from about 8 to about 20 wt% nickel, and from about 5 to about 11 wt% tin, the remaining balance being copper, and having a 0.2% offset yield strength of at least 75 ksi, is used to form a sucker rod coupling or subcoupling. Each coupling is formed from a core having two ends, each end having an internal thread. These box ends engage the pin of a sucker rod or other rod. The exterior surface of the core includes grooves running between the two ends.

It would be desirable to develop new couplings having improved intrinsic galling resistance as well as other desirable properties such that the coupling and the conduit materials are compatible, meaning they both experience minimal wear during operation, do not require any protective coatings, and reduce the total frictional losses of the pumping system.

### BRIEF DESCRIPTION

The present disclosure relates to couplings made from spinodally-hardened copper alloys, and more specifically a coupling that is inserted between the sucker rod of a sucker rod string and the valve rod bushing of a downhole pump. The couplings can be considered part of the sucker rod string. The couplings have a unique combination of properties including high tensile strength, high fatigue strength, high fracture toughness, galling resistance, and corrosion resistance. This combination of properties delays the occurrence of destructive damage to the couplings and other components in pump systems using such couplings (e.g., sucker rods and conduits), while providing mechanical functionality during hydrocarbon recovery operations. This also extends the useful service life of such components, significantly reducing the costs of equipment used to recover hydrocarbons.

Disclosed herein in various embodiments are couplings for a sucker rod string, comprising a core having a first end, a central portion, and a second end. The first and second end each have an end surface. The first end has a linear taper extending from the central portion inwards and ending at the first end surface. Put another way, the first end surface has a smaller diameter than the central portion. The second end surface of the second end has a rounded edge. The diameter of the first end surface is less than the diameter of the second end surface. The couplings are made from a spinodally-hardened copper-nickel-tin alloy having reduced friction and improved wear resistance, wherein the alloy comprises from about 8 to about 20 wt% nickel, and from about 5 to about 11 wt% tin, the remaining balance being copper and wherein the coupling has a sliding coefficient of friction of less than 0.4 when measured against carbon steel.

The diameter of the first end surface is less than a diameter of the second end surface. In some particular embodiments, a threaded bore runs entirely through the core from the first end to the second end. The threads of the bore may have a Rockwell C hardness (HRC) of about 20 to about 40.

The threaded bore at the first end can be adapted to couple with a valve rod bushing, which may be connected to a downhole pump. The first end surface can abut a shoulder portion of the valve rod bushing. An outer diameter of the coupling may be greater than an outer diameter of the valve rod bushing.

The threaded bore at the second end can be adapted to couple with a sucker rod of the sucker rod string. The second end surface can abut a shoulder portion of the sucker rod. An outer diameter of the coupling may be greater than an outer diameter of the sucker rod.

Also disclosed herein are sucker rod strings according to the appended claims. The sucker rod string comprises a sucker rod including an end having a pin with an external thread and a valve rod bushing including a first end having a pin with an external thread and a second end having a counterbore with an internal thread wherein the valve rod bushing connects to a downhole pump. A coupling is also included, as described above. A threaded bore runs entirely through the core of the coupling from the first end to the second endThe threaded bore at the first end of the coupling is complementary with the external thread of the valve rod bushing, and the threaded bore at the second end of the coupling is complementary with the external thread of the sucker rod. The coupling comprises a spinodally-hardened copper-nickel-tin alloy, wherein the alloy comprises from about 8 to about 20 wt% nickel, and from about 5 to about 11 wt% tin, the remaining balance being copper.

Also disclosed herein are pump systems comprising a downhole pump, a power source for powering the downhole pump; and a rod string located between the downhole pump and the power source. The rod string comprises a sucker rod including an end having a pin with an external thread and a valve rod bushing including an end having a pin with an external thread and a second end having a counterbore with an internal thread, wherein the valve rod bushing connects to a downhole pump. A coupling is also included which is as described above. The threaded bore at the first end of the coupling is complementary with the external thread of the valve rod bushing, and the threaded bore at the second end of the coupling is complementary with the external thread of the sucker rod. The coupling comprises a spinodally-hardened copper-nickel-tin alloy, wherein the alloy comprises from about 8 to about 20 wt% nickel, and from about 5 to about 11 wt% tin, the remaining balance being copper.

For illustrative purpose also disclosed herein in various embodiments are couplings for a sucker rod string, comprising a core having a first end, a central portion, and a second end. The first and second end each have an end surface. The first end has a linear taper extending from the central portion inwards and ending at the first end surface. Put another way, the first end surface has a smaller diameter than the central portion. The second end also has a linear taper extending from the central portion inwards and ending at the second end surface. Put another way, the second end surface has a smaller diameter than the central portion. The couplings are made from a spinodally-hardened copper-nickel-tin alloy.

These and other non-limiting characteristics of the disclosure are more particularly disclosed below.

### BRIEF DESCRIPTION OF THE DRAWINGS

The following is a brief description of the drawings, which are presented for the purposes of illustrating the exemplary embodiments disclosed herein and not for the purposes of limiting the same.
**FIG. 1** is a side cross-sectional view of an exemplary sucker coupling of the present disclosure, having a linear taper on one end and a rounded edge on the other end.
**FIG. 2A** is a partial cross-sectional view showing the engagement of a sucker coupling with a sucker rod and a valve rod bushing that is connected to a downhole pump.
**FIG. 2B** is a side view showing the coupling, sucker rod, and valve rod bushing of **FIG. 2A** in an assembled condition.
**FIG. 3A** is a picture of an exemplary sucker coupling of the present disclosure, having a linear taper on both ends.
**FIG. 3B** is a side cross-sectional view showing the interior of the sucker coupling of **FIG. 3A****.**
**FIG. 4** is a schematic illustration of an embodiment of a pumping system of the present disclosure.
**FIG. 5** is a graph illustrating typical sliding friction coefficients of various materials measured by sliding the material on carbon steel. The y-axis is dimensionless and runs from 0 to 0.8 at intervals of 0.1. From left to right, the materials are nickel alloy, carbon steel, aluminum bronze, and copper-nickel-tin.
**FIG. 6** is a graph illustrating the wear of various materials against a steel shaft. The y-axis is the clearance increase due to wear, in inches. The y-axis runs from 0.000 to 0.050 at intervals of 0.005. The x-axis is the number of wear cycles, in thousands, and runs from 0 to 180 at intervals of 30. The steepest line is for hardened steel, and the shallowest line is for copper-nickel-tin.
**FIG. 7** is a picture of a sucker coupling of the present disclosure, made from a Cu-15Ni-8Sn alloy.

### DETAILED DESCRIPTION

A more complete understanding of the components, processes and apparatuses disclosed herein can be obtained by reference to the accompanying drawings. These figures are merely schematic representations based on convenience and the ease of demonstrating the present disclosure, and are, therefore, not intended to indicate relative size and dimensions of the devices or components thereof and/or to define or limit the scope of the exemplary embodiments.

Although specific terms are used in the following description for the sake of clarity, these terms are intended to refer only to the particular structure of the embodiments selected for illustration in the drawings, and are not intended to define or limit the scope of the disclosure. In the drawings and the following description below, it is to be understood that like numeric designations refer to components of like function.

The singular forms "a," "an," and "the" include plural referents unless the context clearly dictates otherwise.

As used in the specification and in the claims, the term "comprising" may include the embodiments "consisting of" and "consisting essentially of." The terms "comprise(s)," "include(s)," "having," "has," "can," "contain(s)," and variants thereof, as used herein, are intended to be open-ended transitional phrases, terms, or words that require the presence of the named components/steps and permit the presence of other components/steps. However, such description should be construed as also describing compositions or processes as "consisting of" and "consisting essentially of" the enumerated components/steps, which allows the presence of only the named components/steps, along with any impurities that might result therefrom, and excludes other components/steps.

Numerical values in the specification and claims of this application should be understood to include numerical values which are the same when reduced to the same number of significant figures and numerical values which differ from the stated value by less than the experimental error of conventional measurement technique of the type described in the present application to determine the value.

All ranges disclosed herein are inclusive of the recited endpoint and independently combinable (for example, the range of "from 2 grams to 10 grams" is inclusive of the endpoints, 2 grams and 10 grams, and all the intermediate values).

The term "about" can be used to include any numerical value that can vary without changing the basic function of that value. When used with a range, "about" also discloses the range defined by the absolute values of the two endpoints, e.g. "about 2 to about 4" also discloses the range "from 2 to 4." The term "about" may refer to plus or minus 10% of the indicated number.

The present disclosure relates to couplings that are made from a spinodally strengthened copper-based alloy. The copper alloys of the present disclosure are copper-nickel-tin alloys wherein the alloy comprises from about 8 to about 20 wt% nickel, and from about 5 to about 11 wt% tin, the remaining balance being copper. The alloys have a combination of strength, ductility, high strain rate fracture toughness, and galling protection. More particularly, the couplings are contemplated to be artificial lift couplings, sucker rod couplings, or sub-couplings used in the oil and gas industry, particularly for hydrocarbon recovery systems.

In particular, the sucker couplings of the present disclosure are contemplated to be used to join the downhole pump to the sucker rod string. A typical downhole pump has a plunger that is reciprocated inside of a pump barrel by the sucker rod string. The plunger and the barrel include a standing valve and a travelling valve. The plunger is connected to a pump drive rod or valve rod, which is in turn connected to a valve rod bushing, which is connected to the sucker rod string through the sucker coupling.

A sucker coupling **130** according to the present disclosure is illustrated in **FIG.** 1. The sucker rod coupling is used to assemble various components of a sucker rod string. For example, sucker coupling **130** may be used to couple a sucker rod **210** and a valve rod bushing **220** as shown in **FIGS. 3A** and **FIG. 3B** and described below.

The sucker coupling **130** itself is a core **132** having a first end **134,** a central portion **170,** and a second end **136**, each end corresponding to a box and having an internal thread (i.e. a female connector) **138**, **140** for engaging the pin of another component in the sucker rod string. The core has a generally cylindrical shape, with the length being greater than the diameter. Dotted lines **172**, **174** indicate where the central portion **170** joins the first end **134** and the second end **136.** The central portion **170** has outer diameter **175.**

The first end **134** has a first end surface **135.** The first end **134** has a linear taper extending inwards toward the end surface **135.** In other words, the first end **134** is chamfered. Alternatively, the first end surface **135** can be described as having a smaller diameter **144** than the diameter **175** of the central portion **170.** The term "taper" here refers only to the diameter decreasing from the middle to each end, and does not require the change in diameter to occur in any given manner. Here, the taper is linear, , i.e. in a straight line.

The second end **136** has a second end surface **137.** The second end **136** has a rounded edge **139** which transitions into the end surface **137.** The second end surface **137** thus has a diameter **146** which is less than the diameter **175** of the central portion **170,** but greater than the diameter **144** of the first end surface **135.** In particular embodiments, the second end surface diameter **146** is at least one-quarter inch greater than the first end surface diameter **144.** In some specific embodiments, the first end surface diameter **144** is one and five-eighths inches, the second end surface diameter **146** is about 1.9 inches, and the diameter **175** of the central portion is 2 inches.

A bore **142** runs entirely through the core from the first end **134** to the second end **136** along the longitudinal axis **160** of the core. Both internal threads **138**, **140** are located on the surface of the bore. Here, both internal threads have the same box thread size, and are complementary to the external threads on other components of the sucker rod string which may be coupled by the coupling **130.**

As further shown in the cross-sectional view provided by **FIG.** 1, the sucker coupling **130** includes a counterbore **152**, **154** at each end surface **135**, **137.** Put another way, the internal thread does not run all the way to the end surface. The longitudinal axis is also indicated by line **160.** The sucker coupling **130** has a substantially smooth cylindrically curved exterior surface **162** between the end surfaces **134, 136.** In other words, the outer diameter remains constant along the length of the central portion **170.** The outer diameter then decreases at the tapered first end **134** and the rounded edge of second end **136.**

**FIG. 2A** and **FIG. 2B** are side views illustrating the engagement between two components of a sucker rod string with a coupling of the present disclosure. **FIG. 2A** is an exploded, partial cross-section view showing a sucker or stabilizer rod **210** and a valve rod bushing **220** that are coupled together via sucker coupling **130**. **FIG. 2A** and

**FIG. 2B** illustrate the use of a coupling having the geometry of sucker coupling **130** described above and shown in **FIG. 1****.**

The sucker or stabilizer rod **210** includes a rod body **212** and two rod ends (only rod end **214** is shown). The rod end **214** includes an externally-threaded pin (or male connector) **216**; a shoulder **218** adapted to abut the end surface of the coupling; and a drive head **219** which can be engaged by a tool for torqueing and tightening stabilizer rods. The valve rod bushing **220** includes a bushing body **222** and two bushing ends **224**, **225.** The valve rod bushing includes an externally-threaded pin (or male connector) **226** at the first bushing end **224,** and a counterbore **227** at the second bushing end **224**. A shoulder **221** is present between the two bushing ends **224**, **225.** The counterbore **227** has internal threads **228** (i.e. a female connector) located on the surface of the counterbore for engaging the pin of another component in the sucker rod string. A drive head **229** is also included, which can be engaged by a tool for torqueing and tightening the valve rod bushing.

**FIG. 2B** shows the components of **FIG. 2A** in assembled form. That is, the male connector of the stabilizer rod **210** is mated with the female connector at the second end of the sucker coupling **130,** and the male connector of the valve rod bushing **220** is mated with the female connector at the first end of the sucker rod coupling 130. **FIG. 2B** illustrates that the outer diameter of the coupling can be greater than the outer diameter of the rod string components to which the couplings attach, such as the stabilizer rod **210** and the valve rod bushing **220**. This prevents the coupled rod string components from contacting the production tubing (i.e. conduit **411** of **FIG. 4**) surrounding the rod string. In addition, the ends of the valve rod bushing and the stabilizer rod are screwed into the coupling until the coupling abuts the shoulder **218**, **221.**

An additional variation of a sucker coupling **330** according to the present disclosure is shown in **FIG. 3A** and **FIG. 3B. FIG. 3A** is a picture of a sucker coupling **330** for assembling various components of a sucker rod string. **FIG. 3B** is a cross-sectional view of the sucker rod coupling **330** pictured in **FIG. 3A**.

Here, the sucker coupling **330** itself is a core **332** having a first end **334**, a central portion **370**, and a second end **336**, each end corresponding to a box and having an internal thread (i.e. a female connector) **338**, **340** for engaging the pin of another component in the sucker rod string. The core has a generally cylindrical shape, with the length being greater than the diameter. Dotted lines **372**, **374** indicate where the central portion **370** joins the first end **334** and the second end **336.** The central portion **370** has outer diameter **375.**

The first end **334** has a first end surface **335**. The first end **334** has a linear taper extending inwards toward the end surface **335**. In other words, the first end **334** is chamfered. Alternatively, the first end surface **335** can be described as having a smaller diameter **344** than the diameter **375** of the central portion **370**.

The second end **336** has a second end surface **337**. For illustrative purpose it is disclosed that the second end **336** also has a linear taper extending inwards toward the end surface **337**. In other words, the second end **336** is also chamfered. Alternatively, the second end surface **337** can be described as having a smaller diameter **346** than the diameter **375** of the central portion **370.** The first end surface diameter **344** is about the same as the second end surface diameter **346**, both of which are less than the central portion outer diameter **375.** The first end surface diameter **344** and the second end surface diameter **346** are each one and five-eighths inches, and the diameter **375** of the central portion is 2 inches.

As illustrated here, a bore **342** runs entirely through the core from the first end **334** to the second end **336** along the longitudinal axis of the core. Both internal threads **338**, **340** are located on the surface of the bore. Here, both internal threads have the same box thread size, and are complementary to the external threads on other components of the sucker rod string which may be coupled by the coupling **330**. The dimensions of the sucker rods and the various parts of the sucker rod coupling are defined by API Specification 11B, the 27th edition of which was issued in May **201**0.

As further shown in the cross-sectional view provided by **FIG. 3B**, the sucker coupling **330** includes a counterbore **352**, **354** at each end surface **335**, **337**. Put another way, the internal thread does not run all the way to the end surface. The longitudinal axis is also indicated by line **360**. The sucker coupling **330** has a substantially smooth cylindrically curved exterior surface **362** along the central portion **370** of the coupling. The outer diameter then decreases at the chamfered end portions **334, 336.** The central outer diameter of these couplings can be greater than the outer diameter of the rod string components to which the couplings attach, such as stabilizer rods or valve rod bushings. This prevents the coupled rod string components from contacting the production tubing (i.e. conduit **411** of **FIG. 4**) surrounding the rod string.

**FIG. 4** illustrates the various parts of a pump system **400** which utilizes various rod string components described above, such as the sucker couplings. The system **400** has a walking beam **422** that reciprocates a rod string **424** that includes a polished rod portion **425.** The rod string **224** is suspended from the beam for actuating a downhole pump **426** that is disposed at the bottom of a well **428.**

The walking beam **422**, in turn, is actuated by a pitman arm which is reciprocated by a crank arm **430** driven by a power source **432** (e.g., an electric motor ) that is coupled to the crank arm **430** through a gear reduction mechanism, such as gearbox **434**. The power source may be a three-phase AC induction motor or a synchronous motor, and is used to drive the pumping unit. The gearbox **434** converts motor torque to a low speed but high torque output for driving the crank arm **430**. The crank arm **430** is provided with a counterweight **436** that serves to balance the rod string **424** suspended from the beam **422**. Counterbalance can also be provided by an air cylinder such as those found on air-balanced units. Belted pumping units may use a counterweight that runs in the opposite direction of the rod stroke or an air cylinder for counterbalance.

The downhole pump **426** may be a reciprocating type pump having a plunger 438 attached to the end of the rod string **424** and a pump barrel **440** which is attached to the end of tubing in the well **428**. The plunger **438** includes a traveling valve **442** and a standing valve **444** positioned at the bottom of the barrel **440**. On the up stroke of the pump, the traveling valve **442** closes and lifts fluid, such as oil and/or water, above the plunger **438** to the top of the well and the standing valve **444** opens and allows additional fluid from the reservoir to flow into the pump barrel **440**. On the down stroke, the traveling valve **442** opens and the standing valve **444** closes in preparation of the next cycle. The operation of the pump **426** is controlled so that the fluid level maintained in the pump barrel **440** is sufficient to maintain the lower end of the rod string **424** in the fluid over its entire stroke. The rod string **424** is surrounded by a conduit **411** which in turn is surrounded by a well casing **410.** The rod string **424** below the polished rod portion **425** is made of sucker or stabilizer rods **446** that are held together via couplings **448**. Couplings **448** may include the sucker couplings (e.g., **130**, **230**) and valve rod bushings (e.g., **320**) described above.

The connection between the sucker rod and the valve rod bushing is one of the most problematic joints in the sucker rod string. Conventional coupling geometries and materials cause rapid tubing wear due to contact between surfaces combined with the elevated velocity of the well fluid as it exits the pump and flows through the clearance between the production tubing and the coupling between the valve rod bushing and the stabilizer rod. The use of the copper alloys disclosed herein as the material for the couplings of the present disclosure reduces damage to threaded connections due to galling-type wear between coupling and tubing. Moreover, the geometry (e.g., chamfered or rounded ends, large outer diameters) of the presently disclosed couplings prevents high energy contact between the coupling and the inner diameter of the tubing due to misalignment. That is, conventional couplings include sharp edges which are more like to damage components in the event of a high energy contact. Moreover, the geometry of the presently disclosed couplings facilitates the flow of well fluids into the diametrical clearance between the coupling and the tubing.

Additionally, the couplings of the present disclosure, being made from the copper alloys disclosed herein, enable the couplings to act as a dampening device. The dampening is enabled because the copper alloys disclosed herein have a low elastic modulus compared to conventional materials. The dampening allows for the absorption of more energy as the lower face of the valve rod bushing (e.g., bushing end **325** in **FIG. 3A**) impacts other components of the sucker rod string during downward stroke of the pump. This phenomenon reduces the tendency of the mating surface of the upper components of the pump to become heavily cold worked during service. Such cold working can lead to loss of ductility and eventually to cracking, as well as the formation of "extruded" metal protrusions extending outward beyond the as-installed diameter of these components. These protrusions damage the inner diameter of the tubing and the production barrel of the pump. Metal fragments may be created as the protrusions fracture. These fragments can cause severe damage to the working surfaces of the pump and the tubing because they remain the system. The high modulus of resistance of the copper alloys disclosed herein enables the coupling to perform this dampening function without plastically deforming. Rather, the coupling is able to return to its original dimensions after both compression on the downward stroke and tension in the upstroke. In other words, the coupling acts as a solid spring.

Generally, the copper alloy used to form the couplings of the present disclosure has been cold worked prior to reheating to affect spinodal decomposition of the microstructure. Cold working is the process of mechanically altering the shape or size of the metal by plastic deformation. This can be done by rolling, drawing, pressing, spinning, extruding or heading of the metal or alloy. When a metal is plastically deformed, dislocations of atoms occur within the material. Particularly, the dislocations occur across or within the grains of the metal. The dislocations over-lap each other and the dislocation density within the material increases. The increase in over-lapping dislocations makes the movement of further dislocations more difficult. This increases the hardness and tensile strength of the resulting alloy while generally reducing the ductility and impact characteristics of the alloy. Cold working also improves the surface finish of the alloy. Mechanical cold working is generally performed at a temperature below the recrystallization point of the alloy, and is usually done at room temperature.

Spinodal aging/decomposition is a mechanism by which multiple components can separate into distinct regions or microstructures with different chemical compositions and physical properties. In particular, crystals with bulk composition in the central region of a phase diagram undergo exsolution. Spinodal decomposition at the surfaces of the alloys of the present disclosure results in surface hardening.

Spinodal alloy structures are made of homogeneous two phase mixtures that are produced when the original phases are separated under certain temperatures and compositions referred to as a miscibility gap that is reached at an elevated temperature. The alloy phases spontaneously decompose into other phases in which a crystal structure remains the same but the atoms within the structure are modified but remain similar in size. Spinodal hardening increases the yield strength of the base metal and includes a high degree of uniformity of composition and microstructure.

Spinodal alloys, in most cases, exhibit an anomaly in their phase diagram called a miscibility gap. Within the relatively narrow temperature range of the miscibility gap, atomic ordering takes place within the existing crystal lattice structure. The resulting two-phase structure is stable at temperatures significantly below the gap.

The copper-nickel-tin alloy utilized herein preferably includes from about 9.0 wt% to about 15.5 wt% nickel, and from about 6.0 wt% to about 9.0 wt% tin, with the remaining balance being copper. This alloy can be hardened and more easily formed into high yield strength products that can be used in various industrial and commercial applications. This high performance alloy is designed to provide properties similar to copper-beryllium alloys.

More preferably, the copper-nickel-tin alloys of the present disclosure include from about 9 wt% to about 15 wt% nickel and from about 6 wt% to about 9 wt% tin, with the remaining balance being copper. In more specific embodiments, the copper-nickel-tin alloys include from about 14.5 wt% to about 15.5% nickel, and from about 7.5 wt% to about 8.5 wt% tin, with the remaining balance being copper.

Ternary copper-nickel-tin spinodal alloys exhibit a beneficial combination of properties such as high strength, excellent tribological characteristics, and high corrosion resistance in seawater and acid environments. An increase in the yield strength of the base metal may result from spinodal decomposition in the copper-nickel-tin alloys.

The copper alloy (disclosed for illustrative purpose) may include beryllium, nickel, and/or cobalt. In some embodiments, the copper alloy contains from about 1 to about 5 wt% beryllium and the sum of cobalt and nickel is in the range of from about 0.7 to about 6 wt%. In specific embodiments, the alloy includes about 2 wt% beryllium and about 0.3 wt% cobalt and nickel. Other copper alloy embodiments can contain a range of beryllium between approximately 5 and 7 wt%.

In some embodiments, the copper alloy contains chromium. The chromium may be present in an amount of less than about 5 wt% of the alloy, including from about 0.5 wt% to about 2.0 wt% or from about 0.6 wt% to about 1.2 wt% of chromium.

In some embodiments, the copper alloy contains silicon. The silicon may be present in an amount of less than 5 wt%, including from about 1.0 wt% to about 3.0 wt% or from about 1.5 wt% to about 2.5 wt% of silicon.

The alloys of the present disclosure optionally contain small amounts of additives (e.g., iron, magnesium, manganese, molybdenum, niobium, tantalum, vanadium, zirconium, and mixtures thereof). The additives may be present in amounts of up to 1 wt%, suitably up to 0.5 wt%. Furthermore, small amounts of natural impurities may be present. Small amounts of other additives may be present such as aluminum and zinc. The presence of the additional elements may have the effect of further increasing the strength of the resulting alloy.

In some embodiments, some magnesium is added during the formation of the initial alloy in order to reduce the oxygen content of the alloy. Magnesium oxide is formed which can be removed from the alloy mass.

In particular embodiments, the internal threads of the coupling are formed by roll forming, rather than by cutting. This process appears to elongate the grains on the outer surface of the threads. Rolled threads have been found to resist stripping because shear failures must take place across the grain, rather than with the grain. This cold working process also provides additional strength and fatigue resistance. As a result, the internal threads may have a Rockwell C hardness (HRC) of about 20 to about 40. The HRC can vary throughout the thread, and this recitation should not be construed as requiring the entire thread to have the same HRC. In particular embodiments, the HRC of the thread is a minimum of 22. The outer surface of the thread may have an HRC of at least 35.

The alloys used for making the couplings of the present disclosure may have a 0.2% offset yield strength of at least 75 ksi, including at least 85 ksi, or at least 90 ksi, or at least 95 ksi.

The alloys used for making the couplings of the present disclosure may have a combination of 0.2% offset yield strength and room temperature Charpy V-Notch impact energy as shown below in Table 1. These combinations are unique to the copper alloys of this disclosure. The test samples used to make these measurements were oriented longitudinally. The listed values are minimum values (i.e. at least the value listed), and desirably the offset yield strength and Charpy V-Notch impact energy values are higher than the combinations listed here. Put another way, the alloys have a combination of 0.2% offset yield strength and room temperature Charpy V-Notch impact energy that are equal to or greater than the values listed here.

**Table 1.**

| **0.2% Offset Yield Strength (ksi)** | **Ultimate Tensile Strength (ksi)** | **Elongation at break (%)** | **Room Temperature Charpy V-Notch Impact Energy (ft-lbs)** | **Preferred Room Temperature Charpy V-Notch Impact Energy (ft-lbs)** |
|---|---|---|---|---|
| 120 | 120 | 15 | 12 | 15 |
| 102 | 120 | 15 | 12 | 20 |
| 95 | 106 | 18 | 22 | 30 |

Table 2 provides properties of another exemplary embodiment of a copper-based alloy suitable for the present disclosure for use in a sucker rod coupling or subcoupling.

**Table 2.**

| | **0.2% Offset Yield Strength (ksi)** | **Ultimate Tensile Strength (ksi)** | **Elongation at break (%)** | **Charpy V-Notch Impact Energy (ft-lbs)** |
|---|---|---|---|---|
| Average | 161 | 169 | 6 | N/A |
| Minimum | 150 | 160 | 3 | N/A |

The 0.2% offset yield strength and ultimate tensile strength are measured according to ASTM E8. The CVN toughness is measured according to ASTM E23. The rod couplings of the present disclosure can be made using casting and/or molding techniques known in the art.

The couplings made of the spinodally-decomposed copper alloys uniquely have high tensile and fatigue strength in combination with high fracture toughness, galling resistance, and corrosion resistance. The unique combination of properties allows the couplings to satisfy basic mechanical and corrosion characteristics needed while reliably protecting system components from galling damage, thereby greatly extending the lifetime of the system and reducing the risk of unanticipated failure. One result is longer well life between maintenance shutdowns. In addition, overall production is enhanced due to the reduced friction.

Some copper-nickel-tin alloys of the present disclosure have a low sliding coefficient of friction. In some embodiments, the copper-nickel-tin alloy in contact with carbon steel, has a sliding coefficient of friction of less than 0.4. In other embodiments, the copper-nickel-tin alloy has a sliding coefficient of about 0.3 or less, including about 0.2 or less.

In particular embodiments of the present disclosure, a copper-nickel-tin alloy in contact with carbon steel typically has a sliding coefficient of less than 0.2 (including about 0.175 or less). In contrast, a nickel alloy in contact with carbon steel typically has a sliding coefficient of friction of 0.7. Carbon steel in contact with carbon steel typically has a sliding coefficient of 0.6 and aluminum bronze in contact with carbon steel typically has a sliding coefficient of 0.4. The comparison of these values are illustrated in the graph of **FIG. 5**. Thus, it is possible to significantly reduce overall frictional losses in the pumping system.

The reduction in friction also results in less tubing wear. **FIG. 6** is a graph showing the use of three different metals used in bearings in contact with a carburized steel shaft with an average bearing stress at 2,000 psi, and oscillating axial motion with side loading. The y-axis indicates the change in clearance due to wear, with a lower value indicating less wear. As seen here, the copper-nickel-tin alloy wore less (triangles, below 0.010 inches) than aluminum bronze (squares, between 0.015 and 0.020 inches) and hardened steel (diamonds, more than 0.045 inches).

The following examples are provided to illustrate the couplings, processes, and properties of the present disclosure. The examples are merely illustrative and are not intended to limit the disclosure to the materials, conditions, or process parameters set forth therein.

### EXAMPLES

### EXAMPLE 1

Sucker rod couplings made of Cu-15Ni-8Sn alloys were used on rod strings in selected trial wells with L80 carbon steel production tubing (HRC 22-23 hardness). Mean run time before failure (MTBF) for steel couplings was approximately 10 months. When the Cu15Ni8Sn couplings were installed, the MTBF increased five-fold. No evidence of wear or metal transfer was found in inspected Cu15Ni8Sn couplings.

One well was shut down 555 days after the Cu15Ni8Sn couplings were installed due to a pump leak. The tubes used to form the well casing were inspected. 50% of tubes that used steel couplings had ≥ 30% wall loss, whereas 0% of tubes that used the Cu15Ni8Sn couplings had ≥ 30% wall loss. 25% of tubes that used steel couplings had ≥ 30% surface pitting, whereas 0% of tubes that used the Cu15Ni8Sn couplings had ≥ 30% surface pitting. It was calculated that this would increase MTBF of the tubing by at least three (3) times.

### EXAMPLE 2

55 Cu15Ni8Sn couplings were installed in the bottom 1,400 feet of a well. The following information was captured:

**Table 4.**

| | Prior Practice | Cu15Ni8Sn Actual |
|---|---|---|
| Rod/coupling drag coefficient | 0.2 | 0.035 |
| Pump stroke (inches) | 141 | 151 |
| Liquid production (barrels per day) | 233 | 248 |
| Polished rod load (pounds) | 33,000 | 31,570 |

The result of Cu15Ni8Sn coupling use was a 6.4% increase in liquid production. Results for similar experiments showed production increases of 9%, maximum load decrease of 12%, and increased pump stroke of 21%.
It is thus expected that pump stroke increases of about 3% up to about 40%, or about 6% to about 40%, or about 6% to about 30%, or about 3% to about 10%, or about 6% to about 10% should occur due to the use of these copper-nickel-tin alloys (compared to the use of steel).

### EXAMPLE 3

A coupling was made of Cu15Ni8Sn alloy. The coupling is depicted in **FIG. 7**, and has a cross-section as illustrated in **FIG. 3B**. The tapered coupling has an outer diameter of two (2) inches with 3/4-inch rolled threads. The coupling is joined to a valve rod bushing, and acts as a centralizer so that the valve rod bushing does not wear out adjacent tubing.

## Claims

1. A coupling (130,330) for a sucker rod string, comprising:
a core (132,332) having a first end (134, 334), a central portion (170, 370), and a second end (136, 336), the first end and the second end each having an end surface (135, 137),
wherein (A) the first end (134, 334) tapers linearly inwards from the central portion (170, 370) to the first end surface (135), (B) the second end surface (137) has a rounded edge; and (C) wherein a diameter (144) of the first end surface (135) is less than a diameter (146) of the second end surface (137), and
wherein the coupling (130) is made from a spinodally-hardened copper-nickel-tin alloy comprising from 8 to 20 wt% nickel, from 5 to 11 wt% tin, the remaining balance being copper, and has a sliding coefficient of friction of less than 0.4 when measured against carbon steel.

2. The coupling of claim 1, further comprising a threaded bore (142) running entirely through the core (132) from the first end (134) to the second end (136).

3. The coupling of claim 2, wherein the threads of the bore (142) have a Rockwell C hardness (HRC) of 20 ± 10% to 40 ± 10%.

4. The coupling of claim 3, where the first end (134) and the second end (136) each also includes a counterbore (152, 154).

5. The coupling of claim 1, wherein the alloy has a 0.2% offset yield strength of at least 586 MPa (85 ksi).

6. A sucker rod string, comprising:
a sucker rod (210) including an end (214) having a pin with an external thread (216);
a valve rod bushing (220) including a first end (224) having a pin with an external thread (226) and a second end (225) having a counterbore (227) with an internal thread (228), wherein the valve rod bushing (220) connects to a downhole pump (426); and
the coupling of claim 1 wherein a threaded bore runs entirely through the core (132, 332) from the first end (134, 334) to the second end (136, 336);
wherein the threaded bore at the first end (134, 334) of the coupling (130, 330) is complementary with the external thread of the valve rod bushing (220), and the threaded bore at the second end (136, 336) of the coupling (130, 330) is complementary with the external thread of the sucker rod (210).

7. The sucker rod string of claim 6, wherein an outer diameter of the sucker rod (210) is greater than an outer diameter of the valve rod bushing (220).

8. The sucker rod string of claim 6, wherein an outer diameter of the coupling is greater than both an outer diameter of the sucker rod (210) and an outer diameter of the valve rod bushing (220).

9. The sucker rod string of claim 6, wherein the first end surface abuts a shoulder portion of the valve rod bushing (220).

10. The sucker rod string of claim 6, wherein the second end surface (137, 337) abuts a shoulder portion of the sucker rod.

11. The sucker rod string of claim 6 or the coupling of claim 1, wherein the alloy has a 0.2% offset yield strength of at least 517 MPa (75 ksi).

12. The sucker rod string of claim 6 or the coupling of claim 1, wherein the alloy comprises 14.5 wt% to 15.5 wt% nickel, and 7.5 wt% to 8.5% tin, the remaining balance being copper.

13. The sucker rod string of claim 6-or the coupling of claim 1, wherein the alloy has a 0.2% offset yield strength of at least 655 MPa (95 ksi) and a Charpy V-notch impact energy of at least 30 J (22 ft-lbs) at room temperature.

14. A method of extracting a fluid from a well, comprising:
operatively connecting a downhole pump (426) to a motor using a sucker rod string; and
operating the downhole pump (426) using the sucker rod string to extract fluid from the well
wherein the downhole pump (426) includes a valve rod bushing (220) including a first end (224) having a pin with an external thread (226) and a second end (225) having a counterbore (227) with an internal thread (228);
wherein the coupling (130, 230) of claim 1 connects the valve rod bushing (220) to the sucker rod string

15. The method of claim 14, wherein a mean time between failure (MTBF) of the sucker coupling (130) is at least four time greater than the MTBF of a coupling made from L80 carbon steel.

16. A pump system (400) comprising:
a downhole pump (426);
a power source (432) for powering the downhole pump (426); and
a rod string (424) located between the downhole pump (426) and the power source wherein the rod string comprises a sucker rod (210) including an end (214) having a pin with an external thread (216);
a valve rod bushing (220) including a first end (224) having a pin with an external thread (226) and a second end (225) having a counterbore (227) with an internal thread (228), wherein the valve rod bushing (220) connects to a downhole pump (426); and the coupling of claim 1.

## Patentansprüche

1. Kopplung (130, 330) für einen Pumpgestängestrang, umfassend:
einen Kern (132, 332), der ein erstes Ende (134, 334), einen mittleren Teil (170, 370) und ein zweites Ende (136, 336) aufweist, wobei das erste Ende und das zweite Ende jeweils eine Endfläche (135, 137) aufweisen,
wobei (A) sich das erste Ende (134, 334) linear nach innen von dem mittleren Teil (170, 370) zu der ersten Endfläche (135) verjüngt, (B) die zweite Endfläche (137) eine gerundete Kante aufweist, und (C) der Durchmesser (144) der ersten Endfläche (135) kleiner ist als der Durchmesser (146) der zweiten Endfläche (137), und
wobei die Kopplung (130) aus einer spinodal gehärteten Kupfer-Nickel-Zinn-Legierung ausgebildet ist, die zwischen 8 und 20 Gew.-% Nickel, zwischen 5 und 11 Gew.-% Zinn und ansonsten Kupfer umfasst und einen Gleitreibungskoeffizienten von weniger als 0,4 gemessen in Bezug auf Kohlenstoffstahl aufweist.

2. Kopplung nach Anspruch 1, die weiterhin eine Gewindebohrung (142) aufweist, die sich vollständig durch den Kern (132) von dem ersten Ende (134) zu dem zweiten Ende (136) erstreckt.

3. Kopplung nach Anspruch 2, wobei das Gewinde der Bohrung (142) einer Rockwell C-Härte (HRC) von 20 ± 10% bis 40 ± 10% aufweist.

4. Kopplung nach Anspruch 3, wobei das erste Ende (134) und das zweite Ende (136) jeweils auch eine Senkung (152, 154) aufweisen.

5. Kopplung nach Anspruch 1, wobei die Legierung eine 0,2%-Dehngrenze von wenigstens 586 MPa (85 ksi) aufweist.

6. Pumpgestängestrang, umfassend:
ein Pumpgestänge (210) mit einem ersten Ende (214), das einen Zapfen mit einem Außengewinde (216) aufweist,
eine Ventilstangenbuchse (220) mit einem ersten Ende (224), das einen Zapfen mit einem Außengewinde (226) aufweist, und einem zweiten Ende (225), das eine Senkung (227) mit einem Innengewinde (228) aufweist, wobei die Ventilstangenbuchse (220) mit einer Bohrlochpumpe (426) verbunden wird, und
die Kopplung von Anspruch 1, wobei sich eine Gewindebohrung vollständig durch den Kern (132, 332) von dem ersten Ende (134, 334) zu dem zweiten Ende (136, 336) erstreckt,
wobei die Gewindebohrung an dem ersten Ende (134, 334) der Kopplung (130, 330) komplementär ist zu dem Außengewinde der Ventilstangenbuchse (220) und die Gewindebohrung an dem zweiten Ende (136, 336) der Kopplung (130, 330) komplementär ist zu dem Außengewinde des Pumpgestänges (210).

7. Pumpgestängestrang nach Anspruch 6, wobei der Außendurchmesser des Pumpgestänges (210) größer ist als der Außendurchmesser der Ventilstangenbuchse (220).

8. Pumpgestängestrang nach Anspruch 6, wobei der Außendurchmesser der Kopplung größer als der Außendurchmesser des Pumpgestänges (210) und als der Außendurchmesser der Ventilstangenbuchse (220) ist.

9. Pumpgestängestrang nach Anspruch 6, wobei die erste Endfläche gegen einen Schulterteil der Ventilstangenbuchse (220) anstößt.

10. Pumpgestängestrang nach Anspruch 6, wobei die zweite Endfläche (137, 337) gegen einen Schulterteil des Pumpgestänges anstößt.

11. Pumpgestängestrang nach Anspruch 6 oder Kopplung nach Anspruch 1, wobei die Legierung eine 0,2%-Dehngrenze von wenigstens 517 MPa (75 ksi) aufweist.

12. Pumpgestängestrang nach Anspruch 6 oder Kopplung nach Anspruch 1, wobei die Legierung 14,5 Gew.-% bis 15,5 Gew.-% Nickel, 7,5 Gew.-% bis 8,5 Gew.-% Zinn und ansonsten Kupfer aufweist.

13. Pumpgestängestrang nach Anspruch 6 oder Kopplung nach Anspruch 1, wobei die Legierung eine 0,2%-Dehngrenze von wenigstens 655 MPa (95 ksi) und eine Charpy-V-Kerbschlagzähigkeit von wenigstens 30 J (22 ft-lbs) bei Raumtemperatur aufweist.

14. Verfahren zum Extrahieren eines Fluids aus einem Bohrloch, umfassend:
operatives Verbinden einer Bohrlochpumpe (426) mit einem Motor unter Verwendung eines Pumpgestängestrangs, und
Betreiben der Bohrlochpumpe (426) unter Verwendung des Pumpgestängestrangs für das Extrahieren von Fluid aus dem Bohrloch,
wobei die Bohrlochpumpe (426) eine Ventilstangenbuchse (220) mit einem ersten Ende (224), das einen Zapfen mit einem Außengewinde (226) aufweist, und einem zweiten Ende (225), das eine Senkung (227) mit einem Innengewinde (228) aufweist, umfasst,
wobei die Kopplung (130, 230) von Anspruch 1 die Ventilstangenbuchse (220) mit dem Pumpgestängestrang koppelt.

15. Verfahren nach Anspruch 14, wobei die mittlere Zeit zwischen Betriebsausfällen (Mean Time Between Failures bzw. MBTF) des Pumpgestängestrangs (130) wenigstens viermal größer als die MBTF einer aus L80-Kohlenstoffstahl hergestellten Kopplung ist.

16. Pumpsystem (400), umfassend:
eine Bohrlochpumpe (426),
eine Antriebsquelle (432) für das Betreiben der Bohrlochpumpe (426), und
ein Pumpgestänge (424), das zwischen der Bohrlochpumpe (426) und der Antriebsquelle angeordnet ist, wobei das Pumpgestänge eine Pumpstange (210) mit einem Ende, das einen Zapfen mit einem Außengewinde (216) aufweist, umfasst,
eine Ventilstangenbuchse (220) mit einem ersten Ende (224), das einen Zapfen mit einem Außengewinde (226) aufweist, und einem zweiten Ende (225), das eine Senkung (227) mit einem Innengewinde (228) aufweist, wobei die Ventilstangenbuchse (220) mit einer Bohrlochpumpe (426) verbunden wird, und
die Kopplung von Anspruch 1.

## Revendications

1. Accouplement (130,330) pour un train de tiges de pompage, comprenant :
un noyau (132, 332) ayant une première extrémité (134, 334), une partie centrale (170, 370) et une deuxième extrémité (136, 336), la première extrémité et la deuxième extrémité ayant chacune une surface d'extrémité (135, 137),
dans lequel (A) la première extrémité (134, 334) se rétrécit linéairement vers l'intérieur à partir de la partie centrale (170, 370) jusqu'à la première surface d'extrémité (135), (B) la deuxième surface d'extrémité (137) a un bord arrondi ; et (C) dans lequel un diamètre (144) de la première surface d'extrémité (135) est inférieur à un diamètre (146) de la deuxième surface d'extrémité (137), et
dans lequel l'accouplement (130) est fabriqué à partir d'un alliage de cuivre-nickel-étain durci par décomposition spinodale, comprenant de 8 à 20 % en poids de nickel, de 5 à 11 % en poids d'étain, le reste étant du cuivre, et a un coefficient de frottement par glissement inférieur à 0,4 lorsqu'il est mesuré par rapport à de l'acier au carbone.

2. Accouplement selon la revendication 1, comprenant en outre un alésage fileté (142) traversant entièrement le noyau (132) de la première extrémité (134) à la deuxième extrémité (136).

3. Accouplement selon la revendication 2, dans lequel les filets de l'alésage (142) ont une dureté Rockwell C (HRC) de 20 ± 10 % à 40 ± 10 %.

4. Accouplement selon la revendication 3, dans lequel la première extrémité (134) et la deuxième extrémité (136) comprennent également chacune un lamage (152, 154).

5. Accouplement selon la revendication 1, dans lequel l'alliage a une limite d'élasticité conventionnelle à 0,2 % d'au moins 586 MPa (85 ksi).

6. Train de tiges de pompage, comprenant :
une tige de pompage (210) incluant une extrémité (214) dotée d'une goupille avec un filetage extérieur (216) ;
une douille (220) de tige de manoeuvre incluant une première extrémité (224) dotée d'une goupille avec un filetage extérieur (226) et une deuxième extrémité (225) dotée d'un lamage (227) avec un filetage intérieur (228),
dans lequel la douille (220) de tige de manoeuvre se raccorde à une pompe de fond (426) ; et
l'accouplement selon la revendication 1 dans lequel un alésage fileté traverse entièrement le noyau (132, 332) de la première extrémité (134, 334) à la deuxième extrémité (136, 336) ;
dans lequel l'alésage fileté à la première extrémité (134, 334) de l'accouplement (130, 330) est complémentaire du filetage extérieur de la douille (220) de tige de manoeuvre, et l'alésage fileté à la deuxième extrémité (136, 336) de l'accouplement (130, 330) est complémentaire du filetage extérieur de la tige de pompage (210).

7. Train de tiges de pompage selon la revendication 6, dans lequel un diamètre extérieur de la tige de pompage (210) est supérieur à un diamètre extérieur de la douille (220) de tige de manoeuvre.

8. Train de tiges de pompage selon la revendication 6, dans lequel un diamètre extérieur de l'accouplement est supérieur à la fois à un diamètre extérieur de la tige de pompage (210) et à un diamètre extérieur de la douille (220) de tige de manoeuvre.

9. Train de tiges de pompage selon la revendication 6, dans lequel la première surface d'extrémité vient en butée contre une partie d'épaulement de la douille (220) de tige de manoeuvre.

10. Train de tiges de soupape selon la revendication 6, dans lequel la deuxième surface d'extrémité (137, 337) vient en butée contre une partie d'épaulement de la tige de pompage.

11. Train de tiges de pompage selon la revendication 6 ou accouplement selon la revendication 1, dans lequel l'alliage a une limite d'élasticité conventionnelle à 0,2 % d'au moins 517 MPa (75 ksi).

12. Train de tiges de pompage selon la revendication 6 ou accouplement selon la revendication 1, dans lequel l'alliage comprend 14,5 % en poids à 15,5 % en poids de nickel, et 7,5 % en poids à 8,5 % d'étain, le reste étant du cuivre.

13. Train de tiges de pompage selon la revendication 6 ou accouplement selon la revendication 1, dans lequel l'alliage a une limite d'élasticité conventionnelle à 0,2 % d'au moins 655 MPa (95 ksi) et une énergie d'impact Charpy sur éprouvette entaillée en V d'au moins 30 J (22 ft-lbs) à la température ambiante.

14. Procédé d'extraction d'un fluide à partir d'un puits, comprenant :
la liaison opérationnelle d'une pompe de fond (426) à un moteur à l'aide d'un train de tiges de pompage ; et
l'exploitation de la pompe de fond (426) en utilisant le train de tiges de pompage pour extraire le fluide du puits,
dans lequel la pompe de fond (426) inclut une douille (220) de tige de manoeuvre incluant une première extrémité (224) dotée d'une goupille avec un filetage extérieur (226) et une deuxième extrémité (225) dotée d'un lamage (227) avec un filetage intérieur (228) ;
l'accouplement (130, 230) selon la revendication 1 reliant la douille (220) de tige de manoeuvre au train de tiges de pompage.

15. Procédé selon la revendication 14, dans lequel un temps moyen entre défaillances (MTBF) de l'accouplement de pompage (130) est au moins quatre fois supérieur au MTBF d'un accouplement fabriqué en acier au carbone L80.

16. Système de pompe (400) comprenant :
une pompe de fond (426) ;
une source d'énergie (432) destinée à alimenter en énergie la pompe de fond (426) ; et
un train de tiges (424) situé entre la pompe de fond (426) et la source d'énergie ;
dans lequel le train de tiges comprend une tige de pompage (210) incluant une extrémité (214) pourvue d'une goupille avec un filetage extérieur (216) ;
une douille (220) de tige de manoeuvre incluant une première extrémité (224) pourvue d'une goupille avec un filetage extérieur (226) et une deuxième extrémité (225) pourvue d'un lamage (227) avec un filetage intérieur (228), dans lequel la douille (220) de tige de manoeuvre se relie à une pompe de fond (426) ; et l'accouplement selon la revendication 1.
